

Jan. 12, 1932.

O. E. ANDRUS ET AL

1,840,305

OIL REFINING STILL

Filed July 13, 1928

*Fig. 1.*



*Fig. 2.*



*Fig. 3.*



*Fig. 4.*



INVENTORS:

ORRIN E. ANDRUS  
AND SUNE HERMANSON.

BY

*W. F. Woodard*  
ATTORNEY.

## UNITED STATES PATENT OFFICE

ORRIN E. ANDRUS AND SUNE HERMANSON, OF MILWAUKEE, WISCONSIN, ASSIGNEES  
TO A. O. SMITH CORPORATION, OF MILWAUKEE, WISCONSIN, A CORPORATION OF  
NEW YORK

## OIL REFINING STILL

Application filed July 13, 1928. Serial No. 292,376.

Our present invention relates to stills and other vessels and is designed primarily to be used in the oil refining industry; but it may be used equally as well in other types of vessels in which the steel structure forming the equipment is subject to the destructive corrosive action of liquids and gases. The invention resides in an improvement in the manner of constructing the vessel disclosed in our prior application, filed October 29, 1927, Serial No. 229,780, on which Letters Patent No. 1,680,276 were granted August 14, 1928. In producing the structure disclosed in the said prior application, the body of the vessel was first fabricated, and the thin, imperforate sheet constituting the liner therefor was then positioned in the vessel and was joined thereto by electric welding through the liner sheet.

In our further experimentation in this branch of the industry, we have successfully demonstrated that the method of applying the thin lining sheet as disclosed in the said prior application, can be greatly simplified with entirely satisfactory results, and we now present our claim for the improvement.

In carrying out our present invention, we apply to one side of the thick metal backing plates of which the body of the still sections are formed, while in their flat state, thin, imperforate, flat sheets of corrosion resisting metal of the character specified in our prior application. These thin lining sheets have an area co-extensive with that of the thick metal backing plates, and are united thereto preferably by electric resistance welding, while both plates are in their flat state.

The composite plate thus produced is converted into tubular form by bending or curving, and following this operation the ends or edges of the plate are brought into alignment in abutting or contiguous relation. Such ends or edges are then electrically welded on their meeting line, axially of the tube, to constitute a tubular section comprised of a thick packing plate and a thin lining sheet of corrosion resisting material, united in such manner as to produce an integral structure.

A suitable number of such integral sections will be assembled end to end and electrically

welded on their circumferential meeting lines, to produce a vessel of the desired length, and heads will be welded to the ends thereof to complete the structure.

Having thus outlined the nature of our invention, we will now describe the same more fully, and will point out the novel features of the invention in the appended claims.

In the accompanying drawings:

Figure 1 is a perspective view of a composite plate, broken away at the left hand end, constructed in accordance with our improved method.

Fig. 2 is a perspective view of a tubular section, formed by the bending of the flat composite plate shown in Fig. 1.

Fig. 3 is a like view showing the tubular section as welded along the meeting ends of the plate, to form an integral structure.

Fig. 4 is a view in elevation, partly broken out, of a still or vessel constructed in accordance with our improved method.

In carrying out our invention we place upon a thick backing plate of steel 10, a thin, imperforate metal sheet 11 of corrosion resisting metal, such as chromium steel, or any other metal having the necessary resisting properties. We then bond the thin sheet 11 to the backing plate 10 by electrically welding the sheet 11 at frequent and contiguous points, as 12, so as to practically unite the plates into an integral structure.

The composite plate is then rolled, pressed or bent into the form of a tube 13, with the ends of the plate meeting in alinement. On account of the thickness of the metal, and to facilitate welding such ends, when the electric arc is used, a deep and narrow welding groove 14 should be formed at the meeting line. An electric arc at the free end of a metallic weld rod is operated in the groove to fuse the walls thereof, and the groove is filled by the deposit of molten metal flowing from the destructible weld rod, so as to form the welded line 15. The welding operation may be facilitated by placing in the groove, slugs or bars of suitable metal, and fusing such slugs or bars by the electric arc, so that the metal thereof will be incorporated in the welded joint.

A plurality of the tubular sections 13 are then arranged end to end and welded together at their circumferential meeting lines as at 16, so as to produce a tubular structure of the desired length. The vessel is then completed by welding heads 17 thereto. Such heads may be conveniently formed from composite plates of the construction shown in Fig. 1, or they may be formed by first drawing the thick plates into cup shapes, and then applying and welding the thin, imperforate sheet lining thereto. The heads are welded to the ends of the tubular structure, as at 18, by circumferential welds, in the manner before set forth.

Preferably the lining sheets 11 are attached to the backing plates 10 by resistance welding, and this may be effected by spotting or by a roller contact. In any manner of attaching the thin, imperforate lining sheet to the backing plate, the bonding points between the two will be so close together that the connection of the plates will be complete. The composite plates may be rolled, pressed or bent without disturbing the relative positions of the plates, or breaking the bonds which unite them. The more numerous the bonding points 12, the more rapid will be the conduction of heat through the vessel during the operating cycle.

While we have shown the composite plates as converted into annular sections, it will be within the scope of our invention to bend such plates on longitudinal lines into trough-like sections, which latter will be welded together on the meeting lines of their longitudinal edges.

After the tubular structure has been completed as described, the joining lines at the inside of the still or vessel should be overwelded with an arc conducted by a fusible weld rod of metal having the properties of the lining, or otherwise welded or treated, so as to avoid the exposure upon the interior of the vessel of any of the carbon steel of the body structure.

The improved method permits the attainment of the purposes of the invention, that is, applying the non-corrosive liner, in a very expeditious, economical and satisfactory manner. In the bending operation, we have found that the best results are attained when the composite plate is heated to a temperature of about 1300° F. When heated to a lower temperature, it is difficult to avoid creeping of the lining sheet, and a smooth lining cannot be produced. When heated to a higher temperature, the metal of the thick backing plate is unduly softened so that the bonded points are liable to rupture, with the result that the rate of heat conduction is lowered by reason of the disturbance of the bonded points.

In some instances, we propose to reverse or duplicate the operation of surfacing the

thick plates, and apply the lining sheet to the exterior surface of the thick plates in the same manner so as to protect the outer surface of the vessel from attack by destructive agencies.

Having thus described our invention, what we claim and desire to secure by Letters Patent of the United States, is:

1. A method of making a thick walled vessel normally subjected to corrosive action which comprises applying a thin sheet of corrosion resistant metal to the surface of a thick steel base plate, said sheet having a thickness less than the thickness of said steel plate and having a yield point not less than that of the steel plate, uniting by resistance welding distributed contacting portions of the sheet and plate to form a composite plate having a surface of corrosion resistant metal, the relative thickness of said plate and sheet causing the jointure between said sheet and plate to be offset from the medial longitudinal plane of the composite plate, heating a plurality of composite plates so lined to a rolling temperature, bending said heated plates into sections capable of being assembled into a cylindrical body with the liner disposed on the interior surface thereof, assembling and welding said sections edge to edge to complete the body of the vessel, and welding end sections to said body to complete the vessel.

2. A method of making a thick walled vessel normally subjected to corrosive action which comprises applying a thin sheet of corrosion resistant metal to the surface of a thick steel base plate, said sheet having a thickness less than the thickness of said steel plate and having a yield point not less than that of the steel plate, electric resistance spot welding the juxtaposed faces of said sheet and plate at close and contiguous points to thereby form a composite plate having an integral surface of corrosion resistant metal, the relative thickness of said plate and sheet causing the jointure between said sheet and plate to be offset from the medial longitudinal plane of the lined plate, heating a plurality of plates so lined to a rolling temperature, bending said heated plates into sections capable of being assembled into a cylindrical body with the liner disposed on the interior surface thereof, assembling and welding said sections edge to edge to complete the body of the vessel, and welding end sections to said body to complete the vessel.

3. A method of making a thick walled vessel normally subjected to corrosive action which comprises applying a sheet of corrosion resistant chromium alloy to the surface of a thick steel plate, electric resistance spot welding the juxtaposed faces of the sheet and plate at close and contiguous points to thereby form a composite plate having a surface of chromium alloy, the relative thickness of said sheet and plate being such that the jointure

between said sheet and plate is substantially offset from the longitudinal medial plane of the lined plate, bending a plurality of plates so formed into complementary sections capable of being assembled into a cylindrical vessel having a substantially continuous chromium alloy interior surface, and assembling and electrically welding said sections edge to edge to complete the vessel.

10 In testimony whereof, we have signed our names at Milwaukee, this 9th day of July, 1928.

ORRIN E. ANDRUS.  
SUNE HERMANSON.

15

20

25

30

35

40

45

50

55

60

65